

# UNITED STATES PATENT OFFICE.

MISSAK MAROUKE, OF LOUISVILLE, KENTUCKY, ASSIGNOR TO HENRY F. REITZ, OF LOUISVILLE, KENTUCKY.

## FILLING MATERIAL FOR TEETH.

1,215,678.

Specification of Letters Patent. Patented Feb. 13, 1917.

No Drawing.

Application filed July 13, 1916. Serial No. 109,173.

To all whom it may concern:

Be it known that I, MISSAK MAROUKE, citizen of France, residing at Louisville, in the county of Jefferson and State of Kentucky, have invented certain new and useful Improvements in Filling Materials for Teeth, of which the following is a specification.

This invention relates to an improvement 13 in filling material for teeth. Heretofore in the art of dentistry two well known processes of filling teeth with gold have been resorted to, one the common method of plugging and the more recent method of casting 18 or inlaying. In the former method as is well known much time is required in packing the gold in small quantities into the cavity and also the necessity of so fashioning the cavity that the margins will overhang 23 and form a retaining wall for the filling. In the inlaying method, a form of the cavity is taken with suitable wax or plastic material; the form or impression is employed to make a matrix or mold in which the gold 28 or inlay is cast in correspondence with the cavity.

The present invention contemplates the production of a material preferably gold which can be filled into the cavity as the 33 primary form as distinguished from a pattern and thereafter be tempered or treated so that the replica of a cavity in metal is produced for inlaying in the usual manner. It has long been regarded as desirable to 38 fill a tooth cavity with a solid filling of gold or precious metal in a manner similar to that now practised in connection with the ordinary "amalgam" filling, which latter, is quickly and accurately placed in the cavity 43 and there held by overhanging walls or anchorage.

The present invention also contemplates a material which can be filled into a cavity, without overhanging walls, quickly and in 48 a manner similar to that of placing "amalgam" fillings, without the use of a mallet, thereby producing a solid inlay filling which can be cemented in any convenient manner to the walls of the cavity.

53 After experiments and tests it has been ascertained that pure gold if reduced to a fine powdered form by an acid treatment and mixed with a relatively small percentage of mercury and then triturated in a mortar, produces a fine grayish alloyed form of

powder. This material is a basic material representing the present invention.

In procuring the grayish filling powder, a convenient method is that of precipitation, now well known in the art. An acid bath is usually employed for precipitating purposes and the fine powdered gold so precipitated is now procurable in the open market. The precipitate is represented as of pure gold in a finely powdered state. After the powdered gold has been procured it has been found convenient to heat the same with a view of consolidating the mass, but not to melt the same, and in this condition there is added to the consolidated mass of free particles a percentage of mercury. It has been found that 20 dwt. of gold powder when mixed with 4 dwt. of mercury and thoroughly stirred and triturated in a dried condition results in the production of a grayish powdered mass which can be readily placed in capsules or bottles for future use. When it is desired to use the material for filling, it is mixed with mercury in substantial proportions much as the now recognized "amalgam" filling is mixed until the mass becomes more or less plastic. The superfluous mercury is then squeezed out through a chamois and the resultant product is then filled in the cavity conveniently 85 the cavity having been first lined with a layer of thin leaf gold. The filling mass is shaped to the desired contour to represent the destroyed part of the tooth and is then removed so that the inlay thus formed represents a true replica of the missing parts of the tooth. In this condition it is subjected to dry heat conveniently an alcohol flame until the mercury is evaporated leaving a solid inlay without any material or objectionable shrinkage. In this form the inlay is placed in the tooth and there cemented, the surfaces being properly burnished in the usual manner. The inlay has the character of and is a "gold filling" of the proper 90 hardness, and fineness.

Should an extra hard filling be desired a precipitated powdered silver or copper may be added to the powdered gold and treated in a manner similar to that heretofore described. By employing the small percentage of a highly distilled mercury and treating the various particles of the powdered gold or filling material therewith it has been ascertained that a very close compact substan- 100 105 110

tially solid and satisfactory filling can be produced. The powdered substance is in color grayish and it has been found that it can be readily mixed with mercury for the purpose of producing a plastic mass for the filling operation. By the thorough mixing and trituration of the mercury with the dried powdered gold each particle of the filling may be said to be composed of a large 10 per cent. of pure gold and a small per cent. of mercury and it is this dried grayish filling powder which represents the discovery and invention herein referred to.

While mercury preferably highly distilled has been found very satisfactory for pretreating the powdered gold so that the material may be employed when desired, it is to be understood that any other substance which would have the effect of producing a 15 substantially solid filling when employed with the powdered gold may be substituted therefor so that the terms employed in the appended claims are not intended as limiting the invention in that particular.

Having thus described the invention, what is claimed as new and desired to be secured by Letters Patent is:—

1. A dried powdered substance suitable

for a filling for teeth comprising finely divided gold particles mixed with a relatively small amount of mercury. 30

2. A dried powdered substance suitable for filling teeth containing a powdered metallic filling substance associated with a relatively small amount of mercury. 35

3. The method of producing a filling material for teeth consisting in subjecting a body of finely powdered gold to the action of heat, adding to the powdered mass a relatively small amount of mercury and thoroughly triturating the combined mass. 40

4. The method of producing a material for use in filling teeth consisting in adding to a body of dried finely powdered precious metal filling material a relatively small 45 amount of mercury and triturating the mass to cause the mercury to come in contact with the various particles of the metal and maintaining the mass in a dried state after treatment.

In testimony whereof I hereunto affix my signature in the presence of two witnesses.

MISSAK MAROUKE.

Witnesses:

J. E. HUTCHINS,  
GUSTAV A. ELLERKAMP.